

No. 609,460.

Patented Aug. 23, 1898.

E. PEIPERS.

MOLD CHILL.

(Application filed May 31, 1895.)

(No Model.)

*Fig. 1.*



*Fig. 2.*



*Fig. 3.*



*Fig. 6.*



*Fig. 4.*



Witnesses

Karin H. Swartz

A. M. Corwin

Emil Peipers

by Danedell & Danedell

Attorneys

# UNITED STATES PATENT OFFICE.

EMIL PEIPERS, OF SIEGEN, GERMANY.

## MOLD-CHILL.

### SPECIFICATION forming part of Letters Patent No. 609,460, dated August 23, 1898.

Application filed May 31, 1895. Serial No. 551,171. (No model.) Patented in Germany June 15, 1894, No. 79,523; in Belgium June 15, 1894, No. 112,773; in England January 22, 1895, No. 1,523, and in Luxembourg January 29, 1895, No. 2,230.

*To all whom it may concern:*

Be it known that I, EMIL PEIPERS, of Siegen, Germany, have invented a new and useful Improvement in Mold-Chills, (patented in 5 Germany June 15, 1894, No. 79,523; in Belgium June 15, 1894, No. 112,773; in England January 22, 1895, No. 1,523, and in Luxembourg January 29, 1895, No. 2,230,) of which the following is a full, clear, and exact description, reference being had to the accompanying drawings, forming part of this specification, in which—

Figure 1 shows in end elevation my improved mold for casting chilled rolls, &c., 15 during its preparation for casting. Fig. 2 is a vertical axial section thereof. Fig. 3 is a vertical cross-section on a larger scale. Fig. 4 is a partial cross-section on a still larger scale. Fig. 5 is a vertical section on the line 20 V V of Fig. 4, and Fig. 6 is a vertical section of the completed mold in position for casting.

In the drawings, 2 represents the bed of the mold, which is made of metal and has an internal cavity 3 of the size and form required 25 for the finished article. In the inner surface of the mold is formed a series of longitudinal grooves or furrows 4. In preparing the mold for use pieces of rope or other suitable removable filling-strips are set in the furrows 30 and may be confined therein by caps 5, which are applied to the ends of the mold. The mold is then placed on its side, as shown in Fig. 1, on rollers 6 or in other suitable position where it can be rotated on its axis, and 35 a mixture 7 of black-lead and water is introduced into the mold-cavity 3. The mold is then revolved slowly on its axis, so that the black-lead mixture shall coat its inner surface and shall fill the furrows over the rope 40 filling-strips, as shown in Figs. 4 and 5. The black-lead mixture is then allowed to dry, and when it has become sufficiently set the

rope pieces are pulled out lengthwise, so as to leave longitudinal cavities at the bases of the furrows. The mold is then heated so as 45 to dry the black-lead completely, and it is then ready to be set in position for casting, as shown in Fig. 6, and on pouring the metal thereinto the chilled roll or other chilled-surface article for which the mold is adapted is 50 formed in the matrix.

My invention is not limited specifically to the use of black-lead, since other similar refractory compositions may be substituted as equivalents.

The advantages of the invention are that it enables the chilled articles to be cast without surface honeycombs or flaws, and by regulating the thickness of the black-lead coating the degree of hardness of the surface can 60 be determined as desired. The cavities left by withdrawal of the filling-strips afford outlets for the gases which come from the molten metal and from the black-lead coating, and by leading off the gases from the coating 65 prevent the latter from peeling from the sides of the mold.

I claim—

A mold-chill for casting chilled-metal articles, having its inner face provided with furrows or grooves, such inner face being covered with a thin coating of refractory material which extends into the furrows and partially fills the same, leaving a longitudinal cavity along the rear face of said filling in 75 each groove for the escape of gases.

In testimony that I claim the foregoing as my invention I have signed my name in presence of two subscribing witnesses.

EMIL PEIPERS.

Witnesses:

WM. ESSENWEIN,  
ERNESTINE ANDRÉ.